

May 8, 1928.

1,669,024

W. RUNGE

CARBONIZATION OF COAL

Filed Nov. 6, 1924



Patented May 8, 1928.

1,669,024

# UNITED STATES PATENT OFFICE.

WALTER RUNGE, OF EAST ORANGE, NEW JERSEY, ASSIGNOR, BY MESNE ASSIGNMENTS, TO INTERNATIONAL COAL CARBONIZATION COMPANY, A CORPORATION OF DELAWARE.

## CARBONIZATION OF COAL.

Application filed November 6, 1924. Serial No. 748,038.

The invention relates to the carbonization or distillation—in the main partial carbonization or distillation—of coal and/or analogous material and therefore the word "coal" as used herein is to be broadly construed as covering what is commonly known as coal and/or also all solid materials analogous thereto.

The invention particularly pertains to carbonizing processes wherein the solid material undergoes treatment when in finely divided or pulverized form in a manner to produce a partially carbonized or partially distilled residue, frequently referred to as partially distilled coke or partially distilled coal.

According to one aspect of the invention the finely divided material within a carbonizing zone retardingly gravitates counter to but in direct contact with a gaseous carbonizing medium that moves upwardly from a combustion zone of approximately between 1150° F. and 1500° F.

According to another aspect of the invention finely divided coal while in suspension in a carbonizing chamber is directly subjected to the carbonizing effect of hot gases resulting from the inflow or introduction of a limited amount of air to a zone within which the air combusts or burns with some of the materials of the carbonizing zone; in other words, with some of the substances being processed while they are within the carbonizing zone.

According to a still further aspect of the invention the partial carbonization of coal is effected within a carbonizing chamber by causing or insuring a delayed gravitation or settling of the coal while a limited amount of air enters and burns with some of the combustible while still within the chamber for causing and effecting the desired carbonization therein.

According to another aspect of the invention the carbonization of coal is effected by causing a showering of pulverized coal from the upper portion of a carbonization zone and causing a hot elastic fluid, which is maintained due to the combustion of a limited amount of oxygen with some of the combustible while still within the chamber, to move in a manner to delay the settling of the coal particles by gravitation until the hot elastic fluid effects the desired carbonization within

the carbonizing zone of the coal under treatment and while in suspension.

The recitals above expressed are not to be construed as limiting the invention for it will be here noted that the invention comprehends not only the aspects above indicated but also other aspects and objects as will be clear and manifest from the specification hereof.

There will now be described a specific manner of realizing the invention and in conjunction therewith reference will be made to the drawing forming a part of the specification.

The sole figure of said drawing diagrammatically illustrates an apparatus or portion of a plant for performing the invention. According to said figure, coal from a storage space 1 is conveyed to a receiving hopper 2, passed to a drier 3, thence to a second receiving hopper 4 from which it is passed to a pulverizer 5, thence to a third receiving hopper or storage bin 6 within which hopper the dry pulverized coal is stored and from which it is withdrawn.

From the hopper or storage bin 6 the dry pulverized or finely divided coal is by suitable means, as 7, fed or showered into the upper portion of an unobstructed vertically extending carbonizing or distilling zone 8 within a retort or carbonizing chamber 9. The feeder 7 is preferably constructed as shown and serves as a preheater or, in other words, as means for preheating the coal prior to introduction into the distilling zone. This is realized due to the absorption of sensible heat of gases within the top of the retort 9 and which gases surround the feeding means 7.

The construction of the feeding means 7 is such as to supply the coal for treatment to the interior of the retort under conditions whereby the coal will enter the retort without permitting the entrance of any objectionable amount of air or the escape to the atmosphere of gases from within the retort. The coal thus fed—which it is manifest is in the form of fine particles—gravitates but with a retarded gravitation toward the bottom or receiving space 10 of the retort 9. In transit the coal or material under treatment is partially carbonized by upwardly moving hot gases and gradually becomes precipitated as a fine partially carbonized residue on parts of the structure defining the

bottom of the receiving space 10. From the bottom of the retort 9 or the receiving space 10 the partially distilled or partially carbonized residue is withdrawn as desired 3 without permitting the entrance of objectionable air to the interior of the retort or without permitting the objectionable escape of gases to the atmosphere. The means for permitting this withdrawal is indicated by 11 10 and 11<sup>a</sup> as sliding gates and by 11<sup>b</sup> as a screw conveyor.

The heat for maintaining the carbonizing process is supplied at the bottom or lower portion of the carbonizing or distilling zone 15 8, as will hereinafter more clearly appear.

The gases of or resulting from the process pass from said carbonizing zone; in other words, from the interior of the retort as through offtake piping 12 to any suitable gas 20 purifying apparatus indicated as at 13, thence to holder 14 from which it is drawn for any desired use as through valve controlled pipes 15, 16 and 16<sup>a</sup>. Some of the gas from the pipe 16 can, if desired, be conducted through a heat interchanger 17, 25 thence through pipes, as 22, which may be considered as parts of burners.

The plant or apparatus may also employ—but it does not necessarily employ—a 30 gas producer as 18 which can be connected so as to deliver gas to the pipes 22 or to a burner 21. Gas from the producer 18 can, by piping 19, be supplied to the burner 21, or gas from the holder 14 can by piping 20 35 also be supplied to the burner 21. The purpose of said burner 21 is to supply heat, or, in other words, to superheat the gas or air passing through the heat interchanger 17 in transit to the pipes 22, and the products of 40 combustion of the burner 21 can pass through the heat interchanger 17 and therefrom to the atmosphere as by piping 23. Should it be desired, as is frequently the case, to pass only air from the heat interchanger and thence into the retort through 45 pipes 22, this can be accomplished by having the valves at 24 and 25 closed and a valve, as at 26, open thus permitting air to enter the heat interchanger. Of course 50 where the gas from the holder 14 or producer 18 is being superheated, dependent upon the particular process being operated, the valve 26 can be closed. The wall of the retort is indicated as being made hollow, as 55 at 30, and if desired gas introduced as through valve controlled pipes 27, 28 and 29 can be employed to add or maintain a certain temperature within said hollow space 30 of the retort 9 and the products of combustion of the gas thus introduced can traverse said space 30 and finally leave on its way to the stack, as through pipe 31.

The receiving space 10 wherein the precipitated coke lodges or deposits in the construction as shown is below the carbonizing

zone at the base of the retort proper and/or within a dry coke cooling device 32 which in effect becomes a continuation of or lower portion of the retort structure. The coke cooling device is dependent for its function 70 upon the indirect cooling effect of air supplied through the pipe 33 and which after having performed the cooling function passes through pipe 34 and preferably branches, one branch leading through pipe 75 35 directly to the pipe 37 which in turn supplies air (or gas dependent upon the particular valve being open) to the preheater 17, another branch leading through pipe 36 directly to the pipe 22. It will thus be noted 80 that heat absorbed from the coke resulting from the process can be returned to the process.

The construction of the plant or apparatus as a whole is such that the retort can be 85 brought to operative temperature for starting the desired process as by the utilization of gas from the producer 18 or the holder 14, as may be convenient or as may be desired. 90

Reference will now be made to a typical process which may be carried out within the apparatus described in realization of the invention. For example, it may be a process relating to the treating or restarting of coal 95 which when introduced therein in dry pulverized form has the following analysis and a heat value of approximately 13,000 B. t. u. (British thermal units) per pound. This coal we will refer to as raw coal sample "A": 100

Moisture 1.5% (water);

Volatile matter 34% (hydrocarbon volatile content);

Fixed carbon 57.5%;

Ash 7%. 105

The pulverized coal may also have a fineness indicated as follows:

59% passed through a 200 mesh screen (to wit, wire screen having 40,000 openings per square inch). 110

85% passed through a 100 mesh screen.

100% passed through a 40 mesh screen.

Such a coal is fed or showered into the top of the carbonizing chamber 9 which is preferably vertical. The coal thus fed is 115 preferably the only gas making material fed into the top of the carbonizing chamber or retort. In fact the pulverized coal is a solid carbonizable fuel and it may be considered as only solid gas making or carbonizable material fed into the retort. The pulverized coal thus fed is allowed to gravitate in cloud-like form through the carbonizing zone, as 8, until the coal or coal particles has or have lost the desired amount of volatile matter and until the carbonized or partially carbonized residue reaches the receiving space 10 below or at the bottom of the carbonizing zone. The carbonization is effected by heat created at the lower regions 120 125 130

of the carbonizing zone in such quantities that there is a complete union between the oxygen of the air and the combustion supporting ingredients within the zone. In the 5 process when once started and underway this heat is preferably maintained solely due to the introduction of air alone at the lower region of the carbonizing zone in such quantities that in the process when started 10 and under way the air unites and burns with some of the carbon of the coal or combustion supporting ingredients or products thereof, thus introduced as specified into the retort and the uniting and burning of the 15 air and said carbon of the coal and the products or ingredients thereof take place while said carbon of the coal or said products or ingredients still remain in the retort or carbonizing chamber so as to produce a hot 20 zone or zone of combustion at the base or lower portion of the carbonizing zone. There is a complete union of the oxygen of the air with the carbon or other combustion supporting ingredients of the precipitating 25 coal so as to produce or maintain the hot zone or zone of combustion in this lower region and this air is introduced or permitted to enter the combustion zone under controlled conditions through the valve controlled pipes 22 either in a hot condition or 30 without being heated, as desired.

Openings may also surround the delivery end of each of the pipes 22 but in that instance a damper member 22<sup>a</sup> is provided 35 whereby the flow of any air through said openings to the interior of the carbonizing zone is under control. If air only is flowing through pipe 22 then in that instance it is preferable to have the openings regulated 40 by the damper members 22<sup>a</sup> completely closed against the inflow of air or the outflow of gases. However, if gas is flowing inwardly through pipe 22, as is possible under certain phases of the invention, then in that 45 instance air would be supplied as through openings controlled by the damper members 22<sup>a</sup>.

The hot products resulting from the combustion just referred to rise or, in other 50 words, travel in a path counter to that of the gravitating particles whereby the coal being treated is suspended within the carbonizing zone 8 a longer period than would be the case if this counter flow did not exist. In 55 other words, the powdered fuel within the carbonizing zone is heated while in suspension in an elastic fluid which is caused to travel to delay the settling of the particles by gravitation and which is maintained at 60 the necessary temperature by heat supplied within the walls of the zone of carbonization.

As illustrating the retardation or delaying of gravitation of the coal within the carbonizing chamber, it will be pointed out that 65 instead of the coal particles gravitating in

about two seconds, as would be the case if not retarded, the time under retarded conditions for the actual precipitation through this carbonizing zone may be approximately 30 seconds and this is substantially the measure of the time for actual carbonization under the conditions recited. The upflowing gases take on or there become mixed therewith gases of the coal given off during the carbonizing period in the chamber with 70 the result that from the upper regions of the chamber there are conducted or withdrawn the gases of or resulting from the process, to wit, the mixed gases resulting from the distillation process and directly resulting from 75 the combustion in the lower portion of the chamber, modified as to their characteristics by such reactions as take place in the presence of coal being treated or in the presence of one another.

It will also be observed that the hot rising gases, while subjecting the coal under treatment to the carbonizing or distilling action, distil off certain vapors or gases and in each instance forthwith carry those vapors or 80 gases toward and to a cooler zone or zones so as to avoid any substantial cracking or breaking down which would be the case if the distilling vapors or gases were subjected 85 to higher heat treatment in the retort.

According to one mode of carbonization along the lines above outlined, as determined by actual experiments raw coal having the characteristics of sample "A"—reduced 90 to a degree of fineness such that 50% passed through a 200 mesh and all of it passed a 40 mesh—was introduced into the top of a vertical retort. This was at a ratio of 12,000 pounds per hour (ratio variations ranging from 6,000 to 18,000 pounds per 95 hour) into a retort of 6 ft. internal diameter and with a carbonizing zone of 50 ft. high and air was supplied to the bottom of the retort at the rate of 2700 pounds per hour under atmospheric conditions and there was 100 maintained in the lower region of the retort a combustion zone which according to pyrometer readings approximated 1150° F. to 1500° F. which have an estimated average vertical 105 velocity of combustion products just above the combustion zone of approximately 1 $\frac{1}{2}$  feet per second travelling counter to the finely divided coal being treated. The temperature of the offgoing gases when leaving the top of the carbonizing chamber was approximately 110 120 550° F. to 850° F. and this gave an estimated average vertical velocity of the offgoing products of approximately  $\frac{2}{3}$  of a foot per second. The temperature of the gases leaving the hot combustion zone of 1150° F. to 1500° F. was reduced to about 900° F. to 1100° F. 125 about one-third way up the carbonizing zone and about 650° F. to 900° F. at about two-thirds way up, and as above indicated 550° F. to 850° F. at the uppermost portion.

The pressure at the bottom of the carbonizing zone with the damper members 22<sup>a</sup> closed and with only air flowing inwardly from the pipe 22 was slightly positive; for example, 1 inch of water, and at the top about neutral or if anything slightly less than atmospheric. The coal treated as above described had the analysis of the raw coal sample "A". The resulting residue was 10 a partially carbonized product having approximately—

|                 | Per cent. |
|-----------------|-----------|
| Volatile matter | 12        |
| Fixed carbon    | 78        |
| Ash             | 10        |

and constituted by weight approximately 72% of the original coal introduced into the carbonizing chamber.

20 It will be manifest that the processes comprehended by the present invention can be modified along the various lines as (a) according to the characteristics of the coal being treated; (b) according to the characteristics of the resulting product; (c) according to the desired characteristics of the gaseous products; (d) according to the fineness of the coal being treated; and (e) according to the size of the retort or to the 25 temperature conditions of the air introduced. For example, by introducing pre-heated air the character of the resulting gases can be modified for the resulting gases can be made richer than would be the case 30 if preheating were not employed, all other conditions being the same.

It is also possible to modify the processes 35 by introducing air and gases so that the gases combined with the air will supply sufficient heat to support the reaction or so that the introduced gas and some of the coal being treated together will combine with the air to produce heat to support the reaction. In other words, to combust the 40 air introduced into the retort.

Mention is herein made to the bringing 45 of the retort up to heat for operating conditions. It will be readily appreciated, however, that in starting the process the retort 50 should be brought as nearly as possible to the heat conditions maintained in the retort when the process is in normal operation, and to that end the heat may be supplied initially in any suitable manner. With the process 55 started, however, there will gradually come a modification, adjustment or change of the temperatures according to those normally realized as the process functions. Whether or not any outside heat is to be employed 60 may depend upon a specific process desired but in general it may be desirable to cut off all such extraneous heat and it is possible for the process herein described to be sustained by the internal heat created solely 65 within the combustion zone which is at the

bottom of the carbonizing chamber and this by the entrance only of a controlled or limited amount of air to the interior of the retort.

In the operation of the process for regulation of pressure conditions at the bottom and top of the retort there can be employed a pressure fan 25<sup>a</sup> for forcing the air or gas through the heat interchanger 17 and an exhauster 14<sup>a</sup> for pulling the gases through 75 pipe 12 and for forcing the gases into the gas purifying apparatus 13.

The term air as employed herein is to be construed as either air as commonly understood, gas having free oxygen as a component part thereof, or even free oxygen alone.

The invention of this application is adaptable for use in connection with the invention which is the subject matter of application No. 748,037, filed November 6, 1924, and entitled Carbonization of coal.

It will be manifest that the invention of this application may be realized in various forms and manners without departing from the spirit and scope of the claims.

What I claim is:—

1. The process which when once started and underway comprises introducing substantially only finely divided coal into the top portion of a hot carbonizing zone and only a limited amount of air into a hot zone of combustion at the bottom portion of the hot carbonizing zone under conditions whereby the resulting rising products of combustion directly contact with the descending coal being treated so as to distil volatile matter from the coal while in suspension, withdrawing from the top portion of the carbonizing zone mixed gases resulting from the process, and collecting and withdrawing as partially distilled coal the residual precipitated from the carbonizing zone.

2. The process which when once started and underway comprises introducing pulverized coal into the upper portion of a hot carbonizing zone within which the pulverized coal in cloud-like form gravitates but with retarded gravitation toward and into a receiving space below the carbonizing zone, causing a limited supply of air to enter a hot zone of combustion at the lower portion of said carbonizing zone under conditions so as to unite and burn with some of the carbon or other combustion supporting ingredients of the coal and thus maintain said hot zone of combustion and so as to maintain therein temperatures approximating between 1150° F. and 1500° F. and so as to cause resulting products of combustion to rise from the zone of combustion and directly contact with the gravitating coal in suspension so as to distil volatile matter therefrom while the coal is in suspension, withdrawing from the upper portion of the

carbonizing zone the mixed gases resulting from the process, and withdrawing from the receiving space below the zone of combustion the resulting partially distilled precipitated 5 coal.

3. The process which comprises introducing finely divided coal at the upper portion of a hot carbonizing zone and a limited supply of air in the lower portion of said zone 10 under conditions to unite and burn with the carbon or other supporting combustion ingredients of the coal and maintain in the lower regions of the carbonizing zone a zone of combustion approximating 1150° F. to 1500° F. 15 from which the products of combustion rise and directly contact with the gravitating coal particles in suspension and under conditions to distil a substantial portion of the volatile matter from the coal 20 while the coal particles are in suspension, collecting from the upper portion of the carbonizing zone mixed gases resulting from the process, and withdrawing as partially distilled coke the residue precipitated from 25 the carbonizing zone.

4. The process which comprises introducing finely divided coal into the upper portion of an unobstructed carbonizing chamber within which the coal thus introduced 30 gravitates in cloud-like form and is heated while in suspension by rising hot gases which are caused to travel so as to delay the settling of the coal particles by gravitation, said heating being carried out in a carbonizing 35 zone having an average temperature between approximately 850° F. 1175° F. said carbonizing zone having at its lower portion its hottest portion which is between approximately 1150° F. and 1500° F. and from 40 which hottest portion the hot gases rise, said hottest portion being maintained at the stated temperature range by the introduction into said hottest portion of a limited amount of air which unites and burns with the carbon or other combustion supporting ingredients of the coal so as to create the heat and simultaneously produce the hot gases which rise from said hottest portion, withdrawing 45 the gaseous products from the upper portion 50 of the carbonizing chamber, and withdrawing the partially distilled residuum from the lower portion of the carbonizing chamber.

5. The process which comprises introducing dry pulverized coal having a substantial 55 volatile content into the upper portion of a hot carbonizing zone, permitting the coal to settle in cloud-like form downwardly along and from the carbonizing zone but delaying its settling solely by the hereinafter specified 60 hot gases, causing only a limited amount of air to enter the lower portion of the carbonizing zone and in which lower portion the air chemically combines with a portion of the products of the introduced pulverized 65 coal while said products still remain within

the carbonizing zone so as to effect a combustion and thereby produce the hot gases which rise and contact with the pulverized coal being treated under conditions to distil from the latter a substantial percentage of 70 the volatile content of the pulverized coal while in suspension withdrawing the mixed gases resulting from the process, and withdrawing as partially distilled coal the residues precipitated from the carbonizing 75 zone.

6. The carbonizing of coal in a retort providing a carbonizing chamber defining an unobstructed vertically extending carbonizing zone within which the coal is carbonized while in suspension in hot gases which carbonizing of the coal is carried out by a process comprising (a) showering powdered coal into an upper portion of the carbonizing zone of the retort and allowing the coal thus fed to gravitate downwardly in cloud-like form through the carbonizing zone; (b) maintaining the requisite temperatures within the carbonizing zone by heat supplied within the walls of the zone of carbonization, 80

which heat is created and maintained substantially solely by the introduction of air alone in a hot zone of combustion which is at the lower region of the carbonizing zone in such quantities that in the process when once started this air unites and burns with some of the carbon or other combustion supporting ingredients of the precipitating coal while said carbon or other combustion supporting ingredients still remain in the carbonizing chamber, said air being limited in quantity and uniting and burning in the manner specified whereby there is effected a substantially complete union of the oxygen of the air with said carbon or other combustion supporting ingredients so as to maintain said hot zone of combustion from which there is emitted the hot products of combustion which constitute gases that are substantially chemically inert with respect to the coal undergoing carbonization and that leave the hot zone of combustion at temperatures approximately 1150° F. to 1600° F., the height of the retort and the time that the coal undergoing carbonization is in the rising hot gases when modified by the gases distilled from the precipitating coal being 95

such that the temperatures of the gases at the top of and when leaving the carbonizing chamber approximate at least as low as 550° 100 F. to 850° F., the arrangement being such that the hot products of combustion leaving the combustion zone move upwardly counter to the downwardly gravitating cloud of powdered coal so that the latter while it 105 gravitates downwardly moves with a retarded gravitation and so that the particles of coal are heated by and while in suspension in the upwardly moving gases; (c) withdrawing from the upper portion of the car- 110

bonizing zone the products of combustion and the other gases resulting from the process; and (d) removing from the lower portion of the retort in finely divided state the carbonized coal thus produced after it has passed downwardly through the carbonizing zone and after separation from the upwardly moving gases, said upwardly moving gases being maintained hot by heat supplied interiorly of the retort as aforesaid and at a location above the place where the finely divided carbon lodged after precipitation from said upwardly moving gases, the finely carbonized coal after lodgment at the base of the retort being kept free from substantial additional heat while in the retort

7. The carbonizing of coal in a retort providing a carbonizing chamber defining an unobstructed vertically extending carbonizing zone within which the coal is carbonized while in suspension in hot gases which carbonizing of the coal is carried out by a process comprising (a) showering powdered coal into an upper portion of the carbonizing zone of the retort and allowing the coal thus fed to gravitate downwardly in cloud-like form through the carbonizing zone; (b) maintaining the requisite temperatures within the carbonizing zone by heat supplied within the walls of the zone of carbonization, which heat is created and maintained substantially solely by the introduction of air alone in a hot zone of combustion which is at the lower region of the carbonizing zone in such quantities that in the process when once started this air unites and burns with some of the carbon or other combustion supporting ingredients of the precipitating coal while said carbon or other combustion supporting ingredients still remain in the carbonizing chamber, said air being limited in quantity and uniting and burning in the manner specified whereby there is effected a

substantially complete union of the oxygen of the air with said carbon or other combustion supporting ingredients so as to maintain said hot zone of combustion from which there is emitted the hot products of combustion providing upwardly moving hot gases that are substantially chemically inert with respect to the coal undergoing carbonization, the height of the retort and the time that the coal undergoing carbonization is in the upwardly moving gases being such that the carbonization is realized by and while the coal particles are in suspension in the upwardly moving gases which are modified by the gases given off from the coal during the carbonizing thereof and which upwardly moving gases serve to retard the downward gravitation of the coal particles until said carbonization has been effected during suspension of the particles in and the heating of the particles by the upwardly moving gases; (c) withdrawing from the upper portion of the carbonizing zone the mixtures of the products of combustion and the gases resulting from the process; and (d) removing from the lower portion of the retort in finely divided state the carbonized coal thus produced after it has passed downwardly through the carbonizing zone and after separation from the upwardly moving gases, said upwardly moving gases being maintained hot by the heat supplied interiorly of the retort as aforesaid and at a location above the place where the finely divided carbon lodged after precipitation from said upwardly moving gases, the finely carbonized coal after lodgment at the base of the retort being kept free from substantial additional heat while in the retort.

In testimony whereof I have hereunto signed my name.

WALTER RUNGE.